

Nov. 10, 1953

P. TALMEY ET AL

2,658,839

## PROCESS OF CHEMICAL NICKEL PLATING

Filed April 21, 1951

FIG. 1



*INVENTORS*

BY *Paul Talmey*  
*William J. Crehan*

Smith, Allen & Baird,  
Atty:

Patented Nov. 10, 1953

2,658,839

# UNITED STATES PATENT OFFICE

2,658,839

## PROCESS OF CHEMICAL NICKEL PLATING

Paul Talmey, Barrington, and William J. Crehan,  
Hinsdale, Ill., assignors to General American  
Transportation Corporation, Chicago, Ill., a  
corporation of New York

Application April 21, 1951, Serial No. 222,222

11 Claims. (Cl. 117—102)

**1** The present invention relates to processes of chemical nickel plating and more particularly to an improved method of utilizing the bath solutions of nickel plating processes such as those disclosed in the copending applications of Gregoire Gutzeit and Abraham Krieg, Serial No. 194,656, filed November 8, 1950, and of Gregoire Gutzeit and Ernest J. Ramirez, Serial No. 204,424, filed January 4, 1951, and in United States Letters Patent No. 2,532,283, issued to Abner Brenner and Grace E. Riddell on December 5, 1950.

In the Brenner and Riddell patent there is disclosed a batch process for chemically plating with nickel by the use of a plating bath including nickel ions and hypophosphite ions, the concentration of the bath being maintained at a predetermined value by the addition of the reagents of the bath at regular intervals.

In the Gutzeit and Krieg application, there is disclosed a batch process of chemically plating a catalytic material, such as steel, with nickel, by contacting the material with an acid bath containing nickel ions and hypophosphite ions and a buffer. This process is carried on under certain optimum conditions which are as follows: The ratio between nickel ions and hypophosphite ions in the bath, expressed in molar concentrations, is within the range 0.25 to 0.60; the absolute concentration of hypophosphite ions in the bath, expressed in mole/liter, is within the range 0.15 to 0.35; the absolute concentration of the buffer in the bath is approximately equivalent to two carboxyl groups for every nickel ion that can be deposited, for instance, in the case of sodium acetate, 0.120 mole/liter of acetate ion; the initial pH of the bath is within the approximate range 4.5 to 5.6; the temperature of the bath is slightly below the boiling point thereof, about 99° centigrade; and the ratio between the volume of the bath, expressed in cm.<sup>3</sup>, and the surface area of the material that is to be plated, expressed in cm.<sup>2</sup>, V/A, is not greater than 10. The buffers mentioned in this application and employed in the test therein referred to are soluble acetates, such as sodium acetate.

In the Gutzeit and Ramirez application, there is disclosed a batch process of chemically plating a catalytic material, such as steel, with nickel, by contacting the material with a bath containing nickel ions and hypophosphite ions and an exaltant in the form of a simple short chain saturated aliphatic dicarboxylic acid. This process is also carried on under certain optimum conditions: The ratio between nickel ions and hypophosphite ions in the bath, expressed in

5 molar concentrations, is within the range 0.25 to 1.60; the absolute concentration of hypophosphite ions in the bath, expressed in mole/liter, is within the range 0.15 to 1.20; the absolute concentration of the exaltant in the bath is approximately equivalent to two carboxyl groups for every nickel ion that can be deposited, for instance, in the case of sodium succinate, at least 0.05 mole/liter of succinate ion; the initial pH of the bath is within the approximate range 4.3 to 6.8; the temperature of the bath is slightly below the boiling point thereof, about 99° C. at atmospheric pressure; and the ratio between the volume of the bath, expressed in cm.<sup>3</sup>, and the surface area of the material that is to be plated, expressed in cm.<sup>2</sup>, V/A, is not greater than 10. The exaltants mentioned in this application and employed in the test therein referred to are soluble salts of malonic, succinic, glutaric, and adipic acids.

In these copending applications, it was pointed out that the plating reaction involved, represented, for instance, by the equation:



25 (1) results in a rapid increase of the hydrogen ion concentration in the bath and may be measured by the corresponding decrease in the pH of the bath. Also it was shown that such an increase in acidity of the bath will considerably slow down the rate of nickel plating and eventually stop the reaction altogether, because the reducing power of the hypophosphite ion is impaired at low pH values and the dissolution rate of the nickel coating or plating in the strongly acid bath will approach and eventually equal the rate of deposition of the nickel.

Moreover, it was pointed out that in order to obtain high nickel plating rates, these processes must be carried out within the optimum pH ranges of the specific baths, and that in order to retard or prevent the formation of black precipitate in the baths, the ratio between the volume of the bath, expressed in cm.<sup>3</sup>, and the surface area of the catalytic material that is to be plated, expressed in cm.<sup>2</sup>, V/A, should be kept below 10.

On the other hand, in any batch or static system without regeneration, there is a limit to the thickness of the nickel coat which may be plated while maintaining a high quality thereof.

Further, the rate of plating decreases as the bath is exhausted, with the consequence that a much longer time is required to obtain an equal increment of thickness near the end of the process than in the beginning. Practically speaking, the ultimate thickness obtainable in a batch or static process is in the range of 0.0005 inch to 0.0010 inch in a period of two hours. The regeneration of the plating bath is unsatisfactory because it has been found that regeneration of a batch bath produces a laminar structure in the coating.

Thus it is of great practical value to be able to deposit any desired thickness of nickel, while the concentrations of the reagents are kept within the optimum ranges mentioned in order to achieve the best quality of plating and the highest plating rate. Insofar as the maintenance of a substantially constant pH is concerned, periodic or continuous addition of a soluble alkali hydroxide or a soluble alkaline salt provides a means of achieving this objective; and, also, this result may be attained by the addition of a buffer salt or a combination of buffers, i. e., compounds comprising the anion of a weakly dissociated acid and a cation able to form a strong base.

The present invention involves improved process steps for maintaining substantially constant the relative and optimum concentrations and proportions of the reagents in the bath, as well as the holding of the pH of the bath within any desired narrow optimum limits, while permitting the plating of any desired thickness of a continuous and homogeneous coating of nickel on the surface area of a catalytic material in a simple and efficient manner. In carrying out the process of the present invention, it may be observed that if the volume of the bath were infinite, while the surface area of the catalytic material to be plated was small, the pH value of the bath would not change, provided sufficient agitation is supplied to avoid any local variation. In other words, if a small object to be plated is placed in a relatively large volume of well agitated bath, the drop in pH due to the plating reaction is so minute as to be practically without effect. On the other hand, it has been found that in a static (as opposed to a dynamic) system, excessive agitation of the bath decreases both the plating rate and the quality of the plating, and that a large ratio of the bath volume to the catalytic material surface area (V/A), tends to favor the formation of black precipitate. Further, and of great importance, a relatively high temperature of the bath tends to favor the formation of black precipitate even in the absence of a catalyst, by spontaneous thermal decomposition. In order to obtain, in addition to other things, the advantage of a large volume of available bath without encountering the disadvantage of a V/A ratio outside of the optimum range, the plating operation proper, according to the present invention, is carried out in a relatively small insulated and heated plating chamber, through which the bath, first preheated to the proper temperature, flows at a relatively low rate, a much larger proportion of the bath being stored in a relatively large reservoir at a substantially lower temperature at which the rate of thermal decomposition is low, for example, substantially at room temperature or even higher. The overflow from the plating chamber is returned directly to the reservoir for re-use; and when the solution in the reservoir is partly

exhausted, it may be regenerated by the periodic or continuous addition of the contained reagents.

It is therefore the primary object of the present invention to provide an improved chemical nickel plating process of the character described in which the plating reaction involved is carried out continuously in a dynamic system and more efficiently and more nearly uniform than theretofore, thereby rendering the process more desirable from a commercial standpoint.

Another object of the invention is to provide an improved process of the character indicated that is continuous so that a substantially uniform and homogeneous nickel coating of any desired thickness may be deposited upon the surface area of a catalytic material that is to be plated.

A further object of the invention is to provide an improved process of the character indicated employing a given nickel plating bath, wherein the bulk of the bath as a substantially inactive solution is stored in a reservoir at a temperature substantially lower than that of the bath in the plating chamber, a small portion of the solution as a plating bath is held at an elevated temperature in a plating chamber, and the solution is circulated at a low rate from the reservoir to the plating chamber and then back to the reservoir, whereby random chemical reduction of the nickel ions in the bath and the consequent formation of black precipitate is eliminated or greatly minimized.

These and other objects and advantages of the present invention will be understood from the foregoing and following description taken with the accompanying drawing, in which Figure 1 is a schematic diagram of an arrangement of apparatus for carrying out the process of the present invention.

Referring now to Fig. 1, the dynamic system there illustrated comprises a reservoir 10 containing a large volume of the solution 11 and a plating chamber 12 containing a small volume of the bath 13, the lower portion of the reservoir 10 being connected to the lower portion of the plating chamber 12 by a conduit 14. A valve 15 is arranged in the conduit 14 so as to accommodate regulation of the rate of flow of the solution 11 from the reservoir 10 in the bath 13 in the plating chamber 12. The upper portion of the solution 11 in the reservoir 10 is disposed at a suitable elevation above the upper portion of the bath 13 in the plating chamber 12, whereby the flow of the solution 11 through the conduit 14 takes place by the action of gravity, the bath 13 in the plating chamber 12 being overflowed from the upper portion thereof into a surrounding launder 16 that communicates via a conduit 17 with a variable speed liquid pump 18. The pump 18 normally returns the overflowed bath 13 via a conduit 19 to the upper portion of the solution 11 in the reservoir 10; and the conduit 19 is also connected via a normally closed valve 20 to a draw-off conduit 21. The intermediate portion of the conduit 14 is provided with a serpentine section 14a that is enclosed by a jacket 22; and the wall of the plating chamber 12 is provided with a surrounding jacket 23. The jackets 22 and 23 are arranged in communicating relation; steam is supplied via a pipe 24 into the heating chambers defined by the jackets 22 and 23; and condensate is removed from these heating chambers via a pipe 25. Thus the solution 11 in the serpentine section 14a of the conduit 14 is preheated to the

temperature required by any particular plating bath prior to the introduction thereof into the plating chamber 12; and the bath 13 contained in the plating chamber 12 is heated to maintain the temperature noted.

A heat exchanging device is shown at 28 which is utilized to reduce the temperature of the bath before it is reintroduced into the storage chamber 11. In small systems this cooling device may be eliminated as the natural cooling effect of the parts 17, 18, 19 and 10 may suffice.

The catalytic material that is to be plated with the nickel is immersed in the bath 13 in the plating chamber 12, and is withdrawn therefrom after a time interval corresponding to the thickness or weight of the nickel coating or plating thereon that is desired. Finally, the reservoir 10 is provided with a drain pipe 26 that is normally closed by an associated valve 27; and of course the component elements of the apparatus or system are formed of noncatalytic materials such as glass, quartz, certain synthetic resins, etc., to prevent the plating of nickel thereon. Thus the major differences between the solution 11 in the reservoir and the bath 13 in the plating chamber are temperature, the presence of a catalytic material, volume and chemical composition. The average chemical composition of the bath 13 and the solution 11 are different to the extent that nickel has been removed and hypophosphite oxidized to the products of its reaction. These differences in composition, however, are by no means as marked as the differences in a batch plating bath between the initiation and conclusion of the plating cycle. The resultant advantages have heretofore been described.

In carrying out any of these processes, the materials that may be coated or plated with nickel include for example such common materials as iron, cobalt, nickel and palladium. Some materials, not catalytic by themselves, can be plated by the use of iron as an initiator. For instance, copper can be used as a basis material, by contacting it with an iron wire to initiate the plating reaction, after which the wire is removed. It should, therefore, be understood that whenever we refer to a catalytic material, we mean thereby a basis material that is catalytic by itself or one that is made catalytic by association with another material. The following elements are examples of noncatalytic materials which ordinarily may not be nickel plated: bismuth, cadmium, tin and lead. Prior to immersing a specimen of catalytic or other basis material to be nickel plated in the bath contained in the plating chamber, the specimen should be first mechanically cleaned to remove any oxide and mill scale; also, the specimen should be degreased and then lightly pickled in a suitable acid, such as HCl.

In carrying out the process of the present invention, employing the apparatus illustrated, and to demonstrate that under these conditions no buffer is needed to produce a good nickel plating, the following tests were performed: baths of the character of that disclosed in the Gutzeit and Krieg application were employed that contained only nickel ions, hypophosphite ions and sodium ions, nickel hydroxide being dissolved in hypophosphorous acid to produce nickel hypophosphite, and sodium hypophosphite being added to obtain the proper concentrations. The pH of the baths were about 3.0 as prepared, and were then adjusted with sodium hydroxide to the optimum

values of 4.5 to 4.6. These baths thus prepared and having the specific compositions noted were employed in the plating of steel samples with the following results:

Table I

| Tests                                                           | No. 1  | No. 2             | No. 3             |
|-----------------------------------------------------------------|--------|-------------------|-------------------|
| Bath composition by analysis:                                   |        |                   |                   |
| Ni <sup>++</sup> mole/liter                                     | 0.0853 | 0.0860            | 0.0862            |
| (H <sub>2</sub> PO <sub>2</sub> ) <sup>-</sup> mole/liter       | 0.261  | 0.2465            | 0.259             |
| pH adjusted to                                                  | 4.61   | 4.61              | 5.51              |
| Test conditions:                                                |        |                   |                   |
| Total volume of bath, liters                                    | 17     | 18                | 18                |
| Volume of plating chamber, cm. <sup>3</sup>                     | 300    | 300               | 300               |
| Area of steel sample cm. <sup>2</sup>                           | 51     | 51                | 51                |
| V/A                                                             |        |                   |                   |
| Average rate of flow, cm. <sup>3</sup> /min.                    | 5.88   | 5.88              | 5.88              |
| Duration of test, time.                                         | 33     | 105               | 114               |
| Temperature, °C                                                 | 97-99  | 97                | 97                |
| Results:                                                        |        |                   |                   |
| Weight of plating, gms.                                         | 2.0281 | 0.730             | 0.593             |
| Rate of plating, $R \times 10^{-4}$ gms./cm. <sup>2</sup> /min. | 0.74   | 0.82              | 0.72              |
| Final pH                                                        | 3.61   | 4.18              | 4.06              |
| Appearance                                                      | Bright | Bright and smooth | Bright and smooth |

From Table I, it may be seen that the rate of nickel plating expressed in gm./cm.<sup>2</sup>/min. is low, but fairly constant, regardless of the rate of flow of the bath and regardless of the length of time of the plating operation.

Much higher rates of nickel plating can be achieved in accordance with the process of the present invention by using a buffer as indicated in the Gutzeit and Krieg application or by employing a bath of the character of that disclosed in the Gutzeit and Ramirez application. For example, using the latter type bath a rate of nickel deposition of  $4.75 \times 10^{-4}$  gms./cm.<sup>2</sup>/min. was achieved.

A very important advantage of the dynamic system of the present process over the batch techniques of the processes of the prior applications and the patent mentioned resides in the circumstance that the chemical composition of the actual plating bath changes very slowly. This results in (1) a very homogeneous composition of the coating which effects a better control of the physical and chemical properties thereof, and (2) a substantially faster plating.

This first result flows from the fact that if any additions are needed to make up for exhaustion of certain reagents, such additions are made in the reservoir thus insuring the constancy of the bath in the plating chamber as will be shown below. The second advantage follows from the first. Because of the constancy of the plating bath in the plating chamber, there is no dilution to any appreciable extent of the amount of nickel to be reduced or of the hypophosphite which does the reducing, thereby eliminating any slowing down of the reaction. Thus the over-all rate of plating is higher. Actually, we have found the rate increase to be even more substantial than could be expected to result from the constancy of the plating solution. It is believed that the laminar flow which helps to remove the hydrogen bubbles has a decided effect in speeding up the rate.

The following tests were carried out in accordance with the process of the present invention employing baths of the character set forth in the Gutzeit and Ramirez application wherein the

7  
solution in the reservoir was periodically regenerated by the addition of small amounts of  $\text{NiCl}_2$  and  $\text{Na}(\text{H}_2\text{PO}_2)$ . These baths thus prepared and having the specific compositions noted were employed in the plating of steel samples with the following results:

Table II

| Tests                                                          | Cycle No. 1      | Cycle No. 3      | Cycle No. 5      | Cycle No. 7      |
|----------------------------------------------------------------|------------------|------------------|------------------|------------------|
| Bath composition by analysis:                                  |                  |                  |                  |                  |
| $\text{Ni}^{++}$ mole/liter                                    | 0.09             | 0.09             | 0.09             | 0.09             |
| $(\text{H}_2\text{PO}_2)^-$ mole/liter                         | 0.225            | 0.225            | 0.225            | 0.225            |
| $(\text{C}_4\text{H}_4\text{O}_4)^-$ mole/liter                | 0.06             | 0.06             | 0.60             | 0.06             |
| pH adjusted to                                                 | 4.48             | 4.61             | 4.50             | 4.50             |
| Test Conditions:                                               |                  |                  |                  |                  |
| Total volume of bath, liters                                   | 2                | 2                | 2                | 2                |
| Volume of plating chamber, cm <sup>3</sup>                     | 65               | 65               | 65               | 65               |
| Area of steel sample, cm <sup>2</sup>                          | 39               | 39               | 39               | 39               |
| V/A                                                            | 1.7              | 1.7              | 1.7              | 2.0              |
| Average rate of flow, cm <sup>3</sup> /min.                    | 49               | 62               | 28               | 34               |
| Duration of test, mins.                                        | 41               | 32               | 37               | 29               |
| Temp., °C                                                      | 97               | 97               | 97               | 97               |
| Results:                                                       |                  |                  |                  |                  |
| Weight of plating, gms.                                        | 0.7499           | 0.6760           | 0.8405           | 0.5350           |
| Rate of plating $R \times 10^{-4}$ , gms/cm <sup>2</sup> /min. | 4.60             | 5.41             | 5.8              | 4.73             |
| Final pH                                                       | 4.22             | 4.36             | 4.35             | 2.5              |
| Appearance                                                     | ( <sup>1</sup> ) | ( <sup>1</sup> ) | ( <sup>1</sup> ) | ( <sup>1</sup> ) |
| Analysis of plating:                                           |                  |                  |                  |                  |
| Percent Ni                                                     | 95.9             | 94.1             | 92.3             | 94.3             |
| Percent P                                                      | 7.4              | 6.97             | 7.64             | 8.9              |

<sup>1</sup> Bright and smooth.

From Table II it will be observed that the specific composition of the nickel-phosphorous coatings through cycle 7 varies only slightly. (Due to the small quantity of coated material relative to basis material, this type of analysis is subject to some variation. The ranges and values given are considered within the analytical error.) Further it is specifically pointed out that this continuous and homogeneous plating produced by the dynamic system of the present invention is entirely different in character from a composite plating that is sequentially built up employing a plurality of batch plating operations of the general character disclosed in the Gutzeit and Krieg application and in the Gutzeit and Ramirez application. It is postulated that this difference resides in the circumstance that when a series of batch plating operations are employed to obtain a relatively thick composite coating, a series of layers of coating are really obtained. In any case, the layers of coating exhibit a stratified characteristic, whereby the coating is not homogenous and uniform throughout either with respect to specific chemical composition in regard to nickel and phosphorous or with respect to hardness and other physical properties. When the article to be plated remains in the bath but periodic additions are made to the plating bath as in Brenner and Riddell, there is an entirely different laminar structure than when employing the method of the present invention.

Moreover, it is noted that the dynamic system of the present invention accommodates the continuous plating of large weights or thick coatings of nickel as compared with the prior batch plating operations. This circumstance is aptly demonstrated by the following test in which there was employed a bath of the general character of that set forth in Gutzeit and Ramirez. This bath thus prepared and having the specific composition noted was periodically regenerated by additions of  $\text{NiCl}_2$  and  $\text{Na}(\text{H}_2\text{PO}_2)$  to the reservoir and was employed in the plating of a steel sample with the following results:

Table III

Bath composition by analysis:

|                                                 |       |
|-------------------------------------------------|-------|
| $\text{Ni}^{++}$ mole/liter                     | 0.09  |
| $(\text{H}_2\text{PO}_2)^-$ mole/liter          | 0.225 |
| $(\text{C}_4\text{H}_4\text{O}_4)^-$ mole/liter | 0.06  |
| pH adjusted to                                  | 4.58  |

Test Conditions:

|                                             |                 |
|---------------------------------------------|-----------------|
| Total volume of bath, liters                | 12.             |
| Volume of plating chamber, cm <sup>3</sup>  | 300.            |
| Area of steel sample, cm <sup>2</sup>       | 103.            |
| V/A                                         | 2.9.            |
| Average rate of flow, cm <sup>3</sup> /min. | 23.             |
| Duration of test, time                      | 5 hrs. 15 mins. |
| Temp., °C                                   | 98.             |

Results:

|                                                            |                    |
|------------------------------------------------------------|--------------------|
| Weight of plating, gms.                                    | 12.1578.           |
| Plating, thickness, mils                                   | 5.                 |
| Plating rate $R \times 10^{-4}$ gms./cm <sup>2</sup> /min. | 3.44               |
| Appearance                                                 | Bright and smooth. |

In conjunction with Table III, it will be specifically observed that over 12 grams of nickel were deposited in this test to form a coating on the steel sample having a thickness of 5 mils. Moreover, there is no critical limitation to the ultimate thickness of the nickel coating that may be deposited, since the solution in the reservoir may be readily periodically or continuously regenerated in the manner previously explained to preserve both the concentrations and proportions of the reagents thereof and also to hold the desired pH thereof, whereby the efficiency of the bath in the plating chamber is constant.

In order to demonstrate that equivalent results may be readily obtained employing samples formed of basis materials, other than steel, a test was conducted employing a bath of the general character of that set forth in the Gutzeit and Ramirez application, wherein the bath was employed in the plating of copper tubing, with the following results.

Table IV

Base material Copper tubing.  
Activation (catalyst) Iron.

Bath composition by analysis:

|                                                                                                  |        |
|--------------------------------------------------------------------------------------------------|--------|
| $\text{Ni}^{++}$ mole/liter as $\text{NiCl}_2$                                                   | 0.067. |
| $(\text{H}_2\text{PO}_2)^-$ mole/liter as $\text{Na}(\text{H}_2\text{PO}_2)$                     | 0.225. |
| $(\text{C}_4\text{H}_4\text{O}_4)^-$ mole/liter as $\text{Na}_2(\text{C}_4\text{H}_4\text{O}_4)$ | 0.06.  |
| pH adjusted to                                                                                   | 4.45.  |

Test conditions:

|                                             |                 |
|---------------------------------------------|-----------------|
| Total vol. of bath, liters                  | 5.              |
| Vol. of plating chamber, cm <sup>3</sup>    | 65.             |
| Area of sample cm <sup>2</sup>              | 21.             |
| V/A                                         | 3.1.            |
| Average rate of flow, cm <sup>3</sup> /min. | 40.             |
| Duration of test, time                      | 2 hrs. 15 mins. |
| Temp., °C                                   | 98.             |

Results:

|                                                               |                    |
|---------------------------------------------------------------|--------------------|
| Weight of plating, gm                                         | 0.9962.            |
| Rate of plating $R \times 10^{-4}$ gms./cm <sup>2</sup> /min. | 3.8.               |
| Appearance                                                    | Bright and smooth. |

The dynamic system of the present invention has also been tested with the use of the Brenner and Riddell bath No. IV given in Table II of their patent with the following results:

Table V

|                                                     |                     |
|-----------------------------------------------------|---------------------|
| Approximate time                                    | 110 minutes.        |
| Volume of solution in reservoir                     | 780 cc.             |
| Volume of plating bath                              | 50 cc.              |
| Area of steel plated                                | 20 cm. <sup>2</sup> |
| Average flow per minute                             | 6 cc./min.          |
| Temperature                                         | 97° C.              |
| Initial pH                                          | 5.05.               |
| Final pH                                            | 4.3.                |
| Weight gain                                         | 0.7483 gm.          |
| Rate $-R \times 10^{-4}$ gms./cm. <sup>2</sup> /min | 3.4.                |
| Appearance                                          | Slightly rough.     |

From the foregoing, it is apparent that great advantages are obtained by the process of the present invention employing the dynamic system in chemical nickel plating of catalytic materials utilizing baths of the general composition set forth in the Brenner and Riddell patent mentioned and in the prior applications of Gutzeit and Krieg and of Gutzeit and Ramirez, or any other chemical nickel plating bath of the same type, particularly with reference to the homogeneous character of the nickel-phosphorous deposits concerning the physical and chemical characteristics thereof and to a greatly increased rate of plating, as well as thickness. Moreover, the dynamic system permits the utilization of a large effective volume of the solution, without the usual formation of black precipitate therein, since the bulk of the solution is stored at a temperature below the initiation of thermal decomposition and only the small portion of plating bath held in the plating chamber is heated to the elevated temperature and in contact with the catalytic material.

It will be understood that the invention is not limited except as defined by the appended claims.

We claim:

1. The continuous process of chemically plating with nickel a solid body essentially comprising an element selected from the group consisting of iron, cobalt, nickel, aluminum, copper, silver, gold, palladium and platinum, which comprises providing an aqueous solution of a nickel salt and a hypophosphite, wherein the ratio between the nickel ions and the hypophosphite ions in said solution is within a first predetermined range and the absolute concentration of the hypophosphite ions in said solution is within a second predetermined range and the pH of said solution is within a third predetermined range, storing the bulk of said solution at a relatively low temperature well below the boiling point thereof in a reservoir, holding a small portion of said solution as a bath at a relatively high temperature slightly below the boiling point thereof in a plating chamber, circulating said solution at a low rate from said reservoir to said plating chamber and then back to said reservoir, heating said solution substantially to said relatively high temperature after withdrawal thereof from said reservoir and before introduction thereof into said plating chamber, cooling said solution substantially to said relatively low temperature after withdrawal thereof from said plating chamber and before return thereof to said reservoir, immersing said body in said bath in said plating chamber, withdrawing said body from said bath in said plating chamber after a time interval corresponding to the thickness of the nickel plating thereon that is desired, and adding during said time interval soluble reagents to said solution in said reservoir to maintain in said bath in said plating chamber during said time interval said ratio and said absolute concentration and said pH respectively in said first and said second and said third predetermined ranges.

2. The continuous process set forth in claim 1, wherein said solution is continuously withdrawn from said reservoir and introduced into the lower portion of said plating chamber and continuously withdrawn from the upper portion of said plating chamber and returned to said reservoir.

3. The continuous process set forth in claim 1, wherein said solution is continuously circulated from said reservoir to said plating chamber and then back to said reservoir, and wherein the volumetric rate of circulation of said solution in cubic feet per minute does not exceed the volume of said bath in cubic feet in said plating chamber.

4. The continuous process of chemically plating with nickel a solid body essentially comprising an element selected from the group consisting of iron, cobalt, nickel, aluminum, copper, silver, gold, palladium and platinum, which comprises providing an aqueous solution of a nickel salt and a hypophosphite and an exaltant, wherein the ratio between the nickel ions and the hypophosphite ions in said solution is within a first predetermined range and the absolute concentration of the hypophosphite ions in said solution is within a second predetermined range and the pH of said solution is within a third predetermined range and the absolute concentration of said exaltant in said solution is at least two carboxyl groups for every nickel ion that can be plated out of said solution, storing the bulk of said solution at a relatively low temperature well below the boiling point thereof in a reservoir, holding a small portion of said solution as a bath at a relatively high temperature slightly below the boiling point thereof in a plating chamber, circulating said solution at a low rate from said reservoir to said plating chamber and then back to said reservoir, heating said solution substantially to said relatively high temperature after withdrawal thereof from said reservoir and before introduction thereof into said plating chamber, cooling said solution substantially to said relatively low temperature after withdrawal thereof from said plating chamber and before return thereof to said reservoir, immersing said body in said bath in said plating chamber, withdrawing said body from said bath in said plating chamber after a time interval corresponding to the thickness of the nickel plating thereon that is desired, and adding during said time interval soluble reagents to said solution in said reservoir to maintain in said bath in said plating chamber during said time interval said ratio and said absolute concentration and said pH respectively in said first and said second and said third predetermined ranges.

5. The continuous process of chemically plating with nickel a solid body essentially comprising an element selected from the group consisting of iron, cobalt, nickel, aluminum, copper, silver, gold, palladium and platinum, which comprises providing an aqueous acid solution of a nickel salt and a hypophosphite, wherein the ratio between the nickel ions and the hypophosphite ions in said solution is within a first range 0.25 to 0.60 and the absolute concentration of the hypophosphite ions expressed in mole/liter in said solution is within a second range 0.15 to 0.35 and the pH of said solution is within a third range 4.5 to 5.6, storing the bulk of said solution at a relatively low temperature well below the

boiling point thereof in a reservoir, holding a small portion of said solution as a bath at a relatively high temperature slightly below the boiling point thereof in a plating chamber, circulating said solution at a low rate from said reservoir to said plating chamber and then back to said reservoir, heating said solution substantially to said relatively high temperature after withdrawal thereof from said reservoir and before introduction thereof into said plating chamber, cooling said solution substantially to said low temperature after withdrawal thereof from said plating chamber and before return thereof to said reservoir, immersing said body in said bath in said plating chamber, withdrawing said body from said bath in said plating chamber after a time interval corresponding to the thickness of the nickel plating thereon that is desired, and adding during said time interval soluble reagents to said solution in said reservoir to maintain in said bath in said plating chamber during said time interval said ratio and said absolute concentration and said pH respectively in said first and said second and said third ranges.

6. The continuous process of chemically plating with nickel a solid body essentially comprising an element selected from the group consisting of iron, cobalt, nickel, aluminum, copper, silver, gold, palladium and platinum, which comprises providing an aqueous acid solution of a nickel salt and a hypophosphite and a simple short chain saturated aliphatic dicarboxylic acid additive, wherein the ratio between the nickel ions and the hypophosphite ions in said solution is within a first range 0.25 to 1.60 and the absolute concentration of the hypophosphite ions expressed in mole-liter in said solution is within a second range 0.15 to 1.20 and the absolute ion concentration of the additive in said solution is at least two carboxyl groups for every nickel ion that can be plated out of said solution and the pH of said solution is within a third range 4.3 to 6.8, storing the bulk of said solution at a relatively low temperature well below the boiling point thereof in a reservoir, holding a small portion of said solution as a bath at a relatively high temperature slightly below the boiling point thereof in a plating chamber, circulating said solution at a low rate from said reservoir to said plating chamber and then back to said reservoir, heating said solution substantially to said relatively high temperature after withdrawal thereof from said reservoir and before introduction thereof into said plating chamber, cooling said solution substantially to said relatively low temperature after withdrawal thereof from said plating chamber and before return thereof to said reservoir, immersing said body in said bath in said plating chamber, withdrawing said body from said bath in said plating chamber after a time interval corresponding to the thickness of the nickel plating thereon that is desired, and adding during said time interval soluble reagents to said solution in said reservoir to maintain in said bath in said plating chamber during said time interval said ratio and said absolute concentration and said pH respectively in said first and said second and said third ranges.

7. The continuous process of chemically plating with nickel a solid body essentially comprising an element selected from the group consisting of iron, cobalt, nickel, aluminum, copper, silver, gold, palladium and platinum, which comprises providing an aqueous solution of a nickel salt and a hypophosphite, wherein the ratio between

the nickel ions and the hypophosphite ions in said solution is within a first predetermined range and the absolute concentration of the hypophosphite ions in said solution is within a second predetermined range and the pH of said solution is within a third predetermined range, storing the bulk of said solution at a relatively low temperature well below the boiling point thereof in a reservoir, holding a small portion of said solution as a bath at a relatively high temperature slightly below the boiling point thereof in a plating chamber, circulating said solution at a low rate from said reservoir to said plating chamber and then back to said reservoir, heating said solution substantially to said relatively high temperature after withdrawal thereof from said reservoir and before introduction thereof into said plating chamber, cooling said solution substantially to said relatively low temperature after withdrawal thereof from said plating chamber and before return thereof to said reservoir, immersing said body in said bath in said plating chamber, withdrawing said body from said bath in said plating chamber after a time interval corresponding to the thickness of the nickel plating thereon that is desired, adding during said time interval soluble nickel-containing and hypophosphite-containing reagents to said solution in said reservoir to maintain in said bath in said plating chamber during said time interval said ratio and said absolute concentration respectively in said first and said second predetermined ranges, and also adding during said time interval a soluble weak alkali to said solution in said reservoir to maintain in said bath in said plating chamber during said time interval said pH within said third predetermined range.

8. The continuous process of chemically plating with nickel a solid body essentially comprising an element selected from the group consisting of iron, cobalt, nickel, aluminum, copper, silver, gold, palladium and platinum, which comprises providing an aqueous solution of a nickel salt and a hypophosphite and having a predetermined composition, storing the bulk of said solution at a relatively low temperature well below the boiling point thereof in a reservoir, holding a small portion of said solution as a bath at a relatively high temperature slightly below the boiling point thereof in a plating chamber, circulating said solution from said reservoir to said plating chamber and then back to said reservoir, heating said solution substantially to said relatively high temperature after withdrawal thereof from said reservoir and before introduction thereof into said plating chamber, cooling said solution substantially to said relatively low temperature after withdrawal thereof from said plating chamber and before return thereof to said reservoir, immersing said body in said bath in said plating chamber, withdrawing said body from said bath in said plating chamber after a time interval corresponding to the thickness of the nickel plating thereon that is desired, and maintaining substantially said predetermined composition of said bath during said time interval by regenerating said solution during said time interval in said reservoir to compensate for the ingredients of said bath that are exhausted during said time interval in said plating chamber, said regeneration of said solution during said time interval in said reservoir consisting essentially of adding thereto appropriate amounts of soluble nickel-containing and hypophosphite-containing agents,

9. The continuous process set forth in claim 1, wherein said soluble reagents added during said time interval to said solution in said reservoir essentially comprise a nickel salt, an alkaline hypophosphite and a weak alkali.

10. The continuous process of chemically plating with nickel a solid body essentially comprising an element selected from the group consisting of iron, cobalt, nickel, aluminum, copper, silver, gold, palladium and platinum, which comprises providing an aqueous solution of a nickel salt and a hypophosphite and having a predetermined composition, circulating said solution from a reservoir to a plating chamber and then back to said reservoir, heating said solution to a relatively high temperature slightly below the boiling point thereof after withdrawal thereof from said reservoir and before introduction thereof into said plating chamber, cooling said solution to a relatively low temperature well below the boiling point thereof after withdrawal thereof from said plating chamber and before return thereof to said reservoir, immersing said body in the hot portion of said solution in said plating chamber to effect nickel plating on the surface of said body, withdrawing said body from said hot portion of said solution in said plating chamber after a time interval corresponding to the thickness of the nickel plating on the surface of said body that is desired, and

20  
25  
30

maintaining substantially said predetermined composition of said hot portion of said solution during said time interval in said plating chamber by regenerating the cool portion of said solution during said time interval in said reservoir to compensate for the ingredients of said solution that are exhausted during said time interval in said hot portion of said solution in said plating chamber, said regeneration of said cool portion of said solution in said reservoir consisting essentially of adding thereto appropriate amounts of soluble nickel-containing and hypophosphite-containing reagents.

11. The process set forth in claim 10, wherein 15 said relatively high temperature is above 80° C. and said relatively low temperature is substantially below 80° C.

PAUL TALMEY.

WILLIAM J. CREHAN.

References Cited in the file of this patent

UNITED STATES PATENTS

| Number    | Name             | Date          |
|-----------|------------------|---------------|
| 1,587,110 | Fisher           | June 1, 1926  |
| 1,740,979 | Golrick          | Dec. 24, 1929 |
| 1,967,856 | Beckman          | July 24, 1934 |
| 2,265,467 | Alexander et al. | Dec. 9, 1941  |
| 2,430,581 | Pessel           | Nov. 11, 1947 |
| 2,532,283 | Brenner et al.   | Dec. 5, 1950  |